

J. C. ADELL.  
PROCESS OF PREPARING HIGHLY OXIDIZED MANGANESE COMPOUNDS.  
APPLICATION FILED AUG. 20, 1917.

1,318,432.

Patented Oct. 14, 1919.



# UNITED STATES PATENT OFFICE.

JAMES C. ADELL, OF CLEVELAND, OHIO.

## PROCESS OF PREPARING HIGHLY-OXIDIZED MANGANESE COMPOUNDS.

1,318,432.

Specification of Letters Patent. Patented Oct. 14, 1919.

Application filed August 20, 1917. Serial No. 187,044.

To all whom it may concern:

Be it known that I, JAMES C. ADELL, a citizen of the United States, residing at Cleveland, in the county of Cuyahoga and State of Ohio, have invented a certain new and useful Improvement in Processes of Preparing Highly-Oxidized Manganese Compounds, of which the following is a full, clear, and exact description, reference being had to the accompanying drawings.

This invention relates to a method of oxidizing manganese compounds, as for example, in making alkali permanganates from commercial oxids of manganese, or for making pure manganese dioxid from impure manganese oxids. The invention further relates to a method of recovering manganese compounds in a pure and preferably highly oxygenated condition from impure ores containing the same and especially from hematite ores which are frequently contaminated with phosphorus, sulfur and silicon.

The invention also provides a method for purifying iron ores from phosphorus and sulfur. This process has been devised primarily for the treatment of certain large deposits of ore in the Duluth-Superior districts whose composition is approximately:

|    |                                      |     |
|----|--------------------------------------|-----|
| 30 | Fe <sub>2</sub> O <sub>3</sub> ----- | 55% |
|    | MnO <sub>2</sub> -----               | 40% |
|    | Silicon, phosphorus and sulfur-----  | 5%  |

Owing to the phosphorus, this ore is now practically valueless since neither the iron nor the manganese can be secured by any practicable known method without such contamination as to render it useless industrially; and even if the phosphorus were not present, an ore containing the indicated amount of manganese is worth only two or three dollars a ton more than one which is free from manganese; while pure pyrolusite under present market conditions is worth approximately one thousand dollars per ton and has never brought less than two hundred to three hundred dollars. The invention is not, however, restricted to this ore or to this product.

The objects of my invention are the provision of a feasible industrial process for recovering manganese in a commercial scale from an impure ore such as above indicated although not restricted to this particular ore; the provision of a recovery process

whereby such manganese is recovered in a highly oxygenated condition such as a dioxid or permanganate; the provision of a process whereby sulfur, phosphorus and other objectionable elements are entirely removed; the provision of a new, improved, cheap, and expeditious process whereby alkali permanganates can be produced directly from pyrolusite or even from other manganese oxids, whether pure or impure; the provision of a process which when applied to impure hematite ores will yield the hematite in pure condition; the provision of a new and improved method of securing pure manganese dioxid from alkali permanganates; while other objects and advantages will appear as the description proceeds.

In the drawings accompanying and forming a part of this application I have illustrated in a very diagrammatic and somewhat conventional manner the various steps of my improved process. In these drawings Figure 1 represents the dry portion of the process, and Fig. 2 represents the wet portion of the same, it being understood that each is read from left to right in the usual manner.

According to my improved process I first crush the raw ore to a reasonable degree of fineness, preferably between sixty and one hundred mesh. Excessive silica is preferably removed from the ore, either before or after the crushing, by any known or suitable method. A small quantity of silica apparently has no deleterious effect upon the reactions excepting to cause a slight loss of reagent, but excessive silica should be avoided.

I next mix the crushed ore with substantially an equal weight of alkali hydrate. This may consist either of potash or soda or a mixture of the two. In cases where the manganese content is subsequently to be removed and sold separately I prefer to employ a mixture of approximately potassium hydroxid one part and sodium hydroxid nineteen parts in order to facilitate the subsequent fusion. In case the permanganate product is desired one of the pure alkalis, generally the potash, is preferably used. Sodium or potassium carbonate can be employed with results wholly as satisfactory, although with no particular gain in cheapness since water free carbonate costs approximately as much as the hydroxid when the comparative amounts of alkali present are

considered. These ingredients are thoroughly mixed together in any suitable or convenient manner as by a rotary concrete mixer shown at A in Fig. 1 and transferred to a suitable container as indicated conventionally at B. I have shown these containers as consisting of open iron pots capable of holding a few hundred pounds of charge, although in large scale operations I anticipate the possibility 10 of employing a continuous process such as an elongated inclined trough or rotary kiln. When the pot has become charged it is transferred as shown at C to the position shown at D in the top of a furnace E of any suitable construction whereby the pot and contents can be heated to a temperature of six hundred to eight hundred degrees centigrade whereupon the alkali combines with the manganese present to form potassium permanganate, this operation being carried out 20 in contact with the air so as to effect the necessary oxidation. I have shown a blowing tube F projecting into the heated pot and receiving from a blower G a current of air which has previously been heated by passing through the coil H in the furnace stack. After a short time, generally only a few minutes although the time depends upon the amount of the charge and the thoroughness of the blowing, the resulting mass will 30 be found to possess a bright blue color streaked with the brown hematite which has not been permanently altered (although I apprehend that it may have performed an important catalytic function in the reaction).

As soon as the reaction is largely complete, the pot is removed as shown at I to make room for a succeeding pot, and is transferred 40 to the position J, where steam from a tube K is blown therein. This steam has the effect of completing the oxidation to the permanganate condition, of any manganese left unchanged by the air, and my experience is 45 that melts subjected to this steam treatment suffer less loss by decomposition and reversion in subsequent manipulations than those not treated in this manner. However, I do not assert that this steam treatment is imperative, and I am not prepared to offer any 50 explanation of its mode of operation, but merely state the result of my observation, that such a treatment is beneficial but not essential, when certain products such as pure permanganates are desired. The contents of 55 the pot are molten at the time the steam is blown therein, and after the conclusion of the steam treatment the pot is left to cool and its contents to harden as indicated at L.

60 As soon as the pot and its contents have cooled below the boiling temperature of water the mass is lixiviated with hot water. This can be performed in the same vessel if desired, particularly in case the pot be only 65 partially filled with the solidified mixture;

but owing to the fact that the pots are preferably operated rather full and to the further fact that the solidified mixture adheres rather closely to the pot, I preferably immerse the whole receptacle in a tank M of 70 hot water as shown at N, the bottom of the tank being preferably provided with a grating O and with a draw-off hopper P closed by suitable valves Q whereby the precipitated ferric sesquioxid can be drawn off 75 into a car R. The mass in the pot being of a porous nature and the permanganates being highly soluble, the receptacle can soon be removed in inverted condition as shown at S and returned for a succeeding use. 80

The sludge from the bottom of the tank M ordinarily consists of almost pure ferric sesquioxid in a compact granular form, not gelatinous or adherent. It is free from sulfur and phosphorus and largely from 85 silicon, all of which form soluble compounds with the alkalis. If the ore should contain cobalt, nickel, titanium, or the like, these oxids will remain with the iron. Also in case any of the manganese oxid in the 90 original melt were oxidized by the air only to manganate, this manganate would be broken up by the steam into permanganate, alkali hydroxid, and manganese dioxid, the last named then remaining with the iron. 95

The liquid in the tank consists of a concentrated solution of alkali permanganate together with excess of alkali and the sulfur, phosphorus, and silicon salts of that alkali, and, if any aluminum were present in the 100 ore, the aluminate of that alkali. Ordinarily the percentage of these impurities is very small and it is possible to evaporate the solution and crystallize the permanganate in pure form directly. Owing to the fact 105 that the present market price of potassium permanganate is approximately eight thousand dollars a ton this is a desirable termination of the process.

This process of making permanganate 110 need not start with a compound ore as above described. Heretofore permanganate has been made by fusing an alkali hydroxid with manganese dioxid, one of several expensive processes being employed to oxidize 115 the resulting product. My invention provides a greatly cheapened and simplified mode of effecting this oxidation, it being necessary merely to add a quantity of oxid of iron as a catalyst and blow air through 120 the mixture, whereupon prompt and complete oxidation takes place, practically all the manganese coming out as permanganate instead of only two thirds thereof as heretofore. None of the iron appears in the 125 resultant solution; even a sulfocyanid test gives negative results. Furthermore any oxid of manganese will operate equally as well as the dioxid, the carbonate of the alkali will enter the reaction equally as well 130

as the hydroxid, and any oxid of iron can be employed. Previous methods have required from 36 to 48 hours, whereas my process is practically completed in as many 5 minutes.

Similarly the reverse of this process can be used to purify iron ores originally free from manganese, for by melting with alkali with the addition of a quantity of manganese 10 oxid, the impurities can be oxidized to a condition where they will unite with the alkali to form a soluble salt. Iron ores purified by my process should have a peculiar value for electric furnace smelting.

15 In case the supply of permanganate produced by my process should exceed the market demand, my process also provides a mode of reducing it to manganese dioxid of a peculiarly pure and active grade. The 20 concentrated solution is withdrawn through a pipe T to an electrolytic apparatus U where it is electrolyzed in a rapid and preferably continuous manner, which breaks up the permanganate into the alkali hydroxid 25 and manganese dioxid. The former remains in solution and passes off through the pipe V to the evaporating pan W where it is evaporated to dryness ready for a subsequent cycle of operations. The manganese 30 dioxid is precipitated in the electrolysis apparatus in the form of a black sludge or mud which is drawn off from time to time through the pipe X. I prefer the continuous flow type of cell since I find no 35 difficulty owing to recombination of the ingredients, and I preferably place the anodes and cathodes in alternation and close together so as to secure a low internal resistance and a high current density. I carry 40 the electrolysis only to the point necessary to dissociate the permanganate which, owing to the normal instability of the solution, is easily and rapidly effected.

It is well known that dilute permanganate solutions will be decomposed with considerable rapidity when left in contact with the air, and insoluble, complex oxids of manganese being precipitated. However, by employing hot concentrated alkaline solutions I experience little or no loss from this 45 reaction. Also by employing a high current density in the electrolysis together with a high over voltage, I precipitate the manganese in the form of the dioxid. I have 50 used with good results and prefer to employ a current of approximately 5 amperes per square decimeter at a potential of 3 to 10 volts, although I do not restrict myself to this and have not yet ascertained the 55 operative limits of potential and current.

The sulfur, phosphorus and silicon originally present in the ore become dissolved in the alkali solution, and if dissociated by the electrolysis, recombine and pass away 60 with the recovered caustic, leaving the man-

ganese and iron in a pure state. For this and other reasons I find a slight but continuous shrinkage of the caustic, amounting under ordinary conditions to approximately ten per cent. for each cycle. In case the 70 alkali carbonates are employed at first instead of the alkali hydroxids, the effect of the electrolysis is still to recover the alkali as caustic. In fact a mixture of caustic and carbonate can be employed with perfectly 75 satisfactory results.

In case metallic manganese is eventually desired, as for steel making, it is perfectly feasible to operate the electrolytic cell at a lower potential so as to produce a lower 80 oxid of manganese, although I can find no advantage in such a modification comparable with the increased time required.

In fact if the manganese output is desired solely for reduction purposes and not as 85 dioxid or permanganate, I recommend the omission of the steam injection, since the presence of alkali manganate in solution serves only to effect the deposition of lower 90 oxids of manganese, which are even easier 90 to reduce than the dioxid. In this particular case the steam treatment is a detriment as causing some manganese loss in the lixiviating tank.

It will be obvious that my process can be 95 started at any point or stopped at any point, that great varieties of apparatus may be employed and that my invention is limited only by the terms of the annexed 100 claims and the prior state of the art.

Having thus described my invention, what I claim is:—

1. In the process of making alkali permanganates the step which consists in heating an oxid of manganese together with an 105 alkali hydroxid or carbonate in air to low redness in contact with iron oxid.

2. The process of separating manganese 110 oxids from hematite, which contains the steps of heating the powdered ore in contact with alkali hydroxid or carbonate to fusing temperature and stirring air into the mixture.

3. The process of converting alkali manganese into permanganates which consists 115 in stirring air into the fused mixture in the presence of iron oxid.

4. The process of preparing alkali permanganates from manganitic hematite ore which contains the steps of fusing the 120 powdered ore with alkali carbonate or hydroxid, blowing air into the fused mixture, cooling, and lixiviating with water.

5. In the process of making alkali permanganates the steps which consist in fusing an oxid of manganese together with an alkali hydroxid or carbonate in contact 125 with iron oxid and afterward blowing steam into the fused mixture.

6. The process of making alkali perman-

ganates which consists in fusing an oxid of manganese together with an alkali hydroxid or carbonate in contact with iron oxid, introducing air and steam into the fused mixture, cooling, and lixiviating with water.

7. The process of separating the mixed oxids of iron and manganese which consists

in fusing the mixture with an alkali hydroxid or carbonate, stirring air into the fused mixture, cooling, lixiviating the resulting mixture, whereby the manganese is dissolved, and decanting.

In testimony whereof I hereunto affix my signature.

JAMES C. ADELL.